

## 1

3,001,885

MANUFACTURE OF ARTIFICIAL ICICLES  
Joseph R. Ehrlich, 1793 Riverside Drive, New York, N.Y.  
No Drawing. Filed Dec. 24, 1958, Ser. No. 782,672  
9 Claims. (Cl. 106—189)

This invention relates to a viscous liquid composition especially useful in the formation of decorative imitation icicles and to a process for the preparation of these imitation icicles. This application is a continuation-in-part of application Ser. No. 441,647, filed July 6, 1954, now abandoned.

In keeping with the Christmas season, or at least the wintry associations of that season, it is customary to decorate Christmas trees with simulations of the natural phenomena which occur during that season. Such phenomena, of course, include snow and ice. The problems incident to a realistic reproduction of snow have already been solved so that it is possible to create a layer of snow indoors which captures much of the character of the actual. But to date the same cannot be said with respect to ice in the form of icicles. This is so because it is quite difficult to provide something with the properties common to all ice formations, that is, a basic solid material which is colorless, translucent, brilliant, perhaps here and there having an air bubble inclusion, and at the same time provide something which will yield ice formations of variegated size and shape. Both these characteristics should be present in order that the illusion of realism be not destroyed.

Heretofore attempts to meet the problems thus presented have often involved the use of glass and plastic which have been the only material comparable in appearance to ice, but the use of glass or plastic fails to meet the second desideratum alluded to above. Obviously the glass or plastic must be preformed and, in order for its use to be economically feasible, it must be cast. This necessarily means that there are severe limitations as to the number of sizes and shapes which can be made available, since obviously these are ready-made, factory manufactured articles. With such limitations the possibility of achieving the objective of realism disappears.

It is an object of this invention to provide a new material for use in producing icicles in the home which in all of the respects already indicated will be eminently suitable.

Another object of this invention is to provide a viscous solution of certain cellulose esters which are suited for the producing of said artificial icicles.

It is a further object of the present invention to provide a process for making artificial icicles on Christmas trees and the like.

Other and more detailed objects will be apparent from the following description and claims.

The material of the present invention is a liquid of considerably viscosity which can be poured from a bottle or squeezed from a collapsible tube at room temperature. When so discharged from its container over a tree branch or other support, the viscous liquid flows downwards with the depending portion thinning to a point in which condition the icicle "freezes." The product is a self-supporting, free-hanging, non-sticky mass at room temperature. It will be observed that the artificial product, just as in the case of a natural icicle, is held to its support without the use of hooks or other hanging device, being held to its support because it has itself formed about the support.

The "icicle solution" of this invention flows freely at room temperature and normal atmospheric conditions to form a pointed cone of an average length of about 3 to 7 inches, preferably 4 inches, within 1 to 5 seconds when released from a closed container in a quantity of about

## 2

½ oz. The flowing liquid gels spontaneously in mid-air after it has changed to the pointed cone-shaped form of about 4 to 7 inches in length; the solution neither drips nor flows too slowly to form either a thread-like shape nor a lump. The solution develops a skin on the surface quickly which is dry to the touch yet is permeable to the solvent vapors to permit a gradual drying and hardening of the icicles. The solution dries clear without a pattern, without blushing, permanent haze, grain or turbidity.

5 There is a minimum of volumetric shrinkage during the drying process. Since it is to be used as a decoration on Christmas trees, the icicles at anytime, when dry or while still containing solvent, do not sustain a flame when ignited. The solution does not spread an objectionable odor, is not corrosive, poisonous or hazardous to handle.

10 It has been found after considerable experimentation that the objects of the present invention could only be accomplished with a viscous cellulose ester solution meeting certain minimum characteristics. Generally speaking, the viscous solution of the present invention must comprise:

(a) At least a two-component solvent system having an essentially predominantly high evaporation rate.  
15 (b) One of the solvents in the solvent system must have a different rate of evaporation than the other.  
20 (c) The cellulose ester component must contain at least one of the cellulose esters more particularly defined below.

(d) The solution in addition to other properties, must be sufficiently viscous to promote gelling in the time allotted for the formation of the icicle, and, at the same time, it must be sufficiently fluent to permit a free flowing out, so that the icicle can grow to the desired length and end in a point.

25 The solvent blends used in accordance with the present invention are non-inflammable and must be composed of at least two solvents even if one solvent alone would be sufficient to dissolve the cellulose ester. One or both solvents can be co-solvents or secondary solvents, though a blend is preferred containing at least one good primary solvent for the particular cellulose ester. Additional solvents in very small quantities can be co-solvents or even diluents.

30 One solvent of the solvent system must evaporate at a faster rate than any other and the whole solvent system must be of the fast evaporation type to cause the spontaneous gelation of the solution at room temperature and normal atmospheric conditions.

35 The gelation phenomenon noted in connection with the present composition is believed to be due to the change in the viscosity of the solution resulting from the change in the solvent system on exposure to the atmosphere at normal temperatures and pressures. Every cellulose ester of a given acid substitution and molecular weight (average chain length as expressed by intrinsic viscosity) exhibits a definite viscosity if dissolved at a given concentration in a given solvent which is characteristic for said solvent. The same cellulose ester when dissolved in another solvent, all conditions equal (concentration, temperature, etc.), might exhibit an entirely different viscosity. The variations of one and the same cellulose ester in various different solvents are remarkable—from 50% to 10,000% or more, e.g. 9% LL-1 Cellulose Acetate as described at page 4 in "Hercules Cellulose Acetate, Properties and Uses," 1954 edition, published by Hercules Powder Company, having 55.0-56.0 combined acetic acid, dissolved in acetone has a viscosity of 46 cps., compared with 62 cps. in methyl-acetate and 203 cps. in methyl ethyl ketone. If 8 parts of methyl ethyl ketone are mixed with 2 parts of methanol the viscosity of said solution goes down to 70 cps. and in the ratio of 9 methyl ethyl ketone:1 methanol to

62 cps.; always using the same LL-1 cellulose acetate as above in 9% concentration. A cellulose acetate-butyrate having a combined butyryl content of 26% and combined acetyl content of 20.5% and a combined cellulose residue of 53.5%, with 2.5% of it free hydroxyl, in a 15% solution in acetone has a viscosity of 272 cps. (Brookfield) at 25° C., but in ethylene chloride the viscosity is 71,000 cps.

From such examples it is evident that a change in the ratio of the components of a solvent blend changes the solvent characteristics of the blend. Not only the solvent capability is likely to change but also a spontaneous and radical change in viscosity can take place. The changing solvent blend at a certain phase might still be a powerful solvent, yet cause a greatly increased viscosity.

In accordance with the present invention the "icicle" solutions are exposed to air from all sides and change their solvent composition continuously and also become more concentrated. With high vapor pressure solvents the changes in viscosity take place very rapidly within a matter of seconds. For example, methyl-, ethyl- or isopropylalcohol are used as co-solvents in the present composition. In a ratio of about 10% to 25% they lower the viscosity of most cellulose esters in a methylene chloride solution. In ratios of less than 10% and more than 25% they increase the viscosity even beyond the viscosity of a cellulose ester solution in methylene chloride alone. Thus the change is very pronounced. The methylene chloride evaporates faster than the alcohols especially when the right cellulose esters are dissolved.

In a cellulose ester solution which is at the saturation concentration or close to saturation but still flowing, a change in viscosity may cause gelation. However, not all cellulose ester solutions which gel in accordance with this theory can be used for the production of artificial icicles. In order to be usable for this purpose they must meet a number of close specifications. Moreover, plasticizers and modifiers also influence the viscosity and solubility of the blended solute in a solvent or solvent blend and, therefore, must be carefully chosen in order to meet the specifications.

With all these limitations not all cellulose esters, plasticizers, modifiers and solvents can be used even if they behaved "qualitatively" in a similar manner. Thus, for example, if two cellulose acetates "x" and "y" are both soluble in the same solvent but their viscosity figures or saturation rates are different, such cellulose acetates might not be interchangeable for my purpose. The same is true for modifiers, solvents, etc. A plasticizer might be compatible with said ester "x" in a certain ratio which is necessary for my purpose but not compatible in the same ratio with ester "y." For example, cellulose acetate PM-3 such as described at page 4 in "Hercules Cellulose Acetate, Properties and Uses," 1954 edition, published by Hercules Powder Company, in a formulation:

TABLE I

|                                                   | Parts by weight |
|---------------------------------------------------|-----------------|
| Cellulose acetate PM-3                            | 20              |
| Santicizer M-17 (methyl phthalyl ethyl glycolate) | 12              |
| Methylene chloride:ethanol                        | 9:1             |

"Santicizer M-17," as described in "Handbook of Material Trade Names," by Zimmermann and Lavine, 1953 edition, page 500, as methyl phthalyl ethyl glycolate  $C_6H_4(COO)_2CH_3CH_2COOC_2H_5$ , is completely compatible with PM-3 in this ratio and almost in any other ratio. However Aroclor 1254 (chlorinated biphenyl), which is useful for the present purposes, is not compatible with PM-3 in his ratio and, therefore, not interchangeable. The formula in Table I above is too viscous to flow freely and is not useful for the present purpose. The use of this results in a lump and not a pointed icicle. The same formula without the "Santicizer M-17" gives a rippled pattern and slight turbidity with a great deal of shrinkage. This also is not usable for the present pur-

pose. However, as will be noted below, PM-3 may be used in the present invention when blended with other cellulose esters.

In accordance with the present invention the drying "icicle" should shrink in volume as little as possible. Thus there is dissolved only as much solute in the solvent as is consistent with free flow and mutual compatibility. This cannot be effected with just any plasticizer or modifier that is compatible with the respective ester but it must be selected judiciously. The total solute is preferably 40% to 50% by weight of the solution though, with certain bulky cellulose esters, "icicles" on the somewhat "lean" side can be made with a little less solute. Thus the solids content i.e. the non-evaporable part of the solution, may vary from 30% to 50% by weight of the total solution.

The solvent system of this invention constitutes the largest portion of the solutions. It must be non-inflammable and must consist of at least two components with a high but different evaporation rate. The evaporation rates of solvents and solvent systems which are useful for the present purposes are as expressed by vapor pressure roughly between the limits of 30 to 350 mm. mercury at 20° C. Or, if N-butyacetate has an arbitrary evaporation rate of 100, the solvents useful for this invention should have an evaporation rate from 230 to 1200.

Some typical evaporation rates and vapor pressure of solvents that can be used in the present invention can be seen in Table II below:

30

TABLE II

|                     | Relative Evaporation Rates (N-butyacetate=100) | Vapor Pressure, mm. | B.P., °C. | Evaporation time (Ethyl Ether=1) |
|---------------------|------------------------------------------------|---------------------|-----------|----------------------------------|
| 35                  |                                                |                     |           |                                  |
| Methylene chloride  | 1,200                                          | 340-357             | 39-40.1   | 1.8                              |
| Methanol            | 610                                            | 94-95               | 61.7      | 6.3                              |
| Ethanol             | 340                                            | 42                  | 78.5      | 8.3                              |
| Isopropanol         | 230                                            | 31-33               | 80-82     | 21.0                             |
| 40                  | Cyclohexane                                    | ?                   | 77        | ?                                |
| Carbontetrachloride | ?                                              | 81.4                | 76.8      | 4.1                              |
| Ethylene dichloride | ?                                              | 66                  | 83.7      | 4.1                              |

The solvents, co-solvents or diluents which can be used in accordance with the present invention are: methylene 45 chloride, methanol, ethanol, isopropanol, carbontetrachloride, ethylene dichloride and cyclohexane. Only insignificant quantities of diluents may be added. The preferred ratio of methylene chloride: secondary solvent is 9:1, though ratios from 9.3:0.7 to 8.5:1.5 can be used. A 50 ratio of 8:2 is workable as far as "icicle" formation is concerned but not desirable because of flammability.

There are a number of cellulose esters which will dissolve in the solvent blends mentioned herein and yet will not meet all the specifications of this invention and, therefore, are not usable for the present purposes. The useful

cellulose esters are those which are highly soluble in the proper solvent blends as expressed by high concentration at the saturation point and at the same time result in a solution of relatively low viscosity—the viscosity being such that a quantity of about 1/2 oz. of solution flows freely within 1 to 5 seconds to form a pointed cone of an average length of 3 to 7 inches after which time the cone gels. Thus, two factors are important for the choice of the right cellulose esters: solubility and viscosity.

60 Solubility is a function of acid substitution, type of solvent and concentration. Sometimes, e.g., certain cellulose esters are less soluble at a lower concentration than at a higher one. Viscosity depends on the type of ester which, in turn, is a function of acid substitution and chain length (mol. weight) and concentration. As solubility and viscosity also change with temperature, all 65 specifications and information given herein are to be understood at room temperature of 20° C.-25° C.

70 Cellulose acetates which are useful for the present purposes have an acid substitution as expressed by combined

acetic acid of from 54.1% to 56% or an acetyl content from 39-40.35%. The viscosity ranges from 1 to 8 seconds as determined by the falling time of a  $\frac{5}{16}$ " steel ball through 10 in. of a 20% solution by weight of cellulose acetate dissolved in a solvent composed of 90:10 acetone:ethanol (by weight) held in a 1 in. diameter tube at 25° C. (ASTMD 871-48 Formula A).

Cellulose acetates with a higher combined acetic acid content, though being mostly used for solvent casting of films, etc., have even better solubility but, as such, are not usable for the present purposes because all commercial products in this range come in a viscosity grade not suitable for this invention. Also they have more solvent retention.

However, it is admissible to blend different grades of cellulose acetates or cellulose acetate with the more compatible cellulose acetate-butyrate to obtain an intermediate viscosity grade. However, it is best that such blends of cellulose acetates be made of grades showing not more than fivefold variation in viscosity in order to avoid grain formation. It is also possible to blend small portions of cellulose acetates with combined acetic acid content of less than 54.1 or more than 56.0 with larger portions of the cellulose acetates with 54.1-56.0 combined acetic acid as long as the flow and gel characteristics necessary for the present purposes are obtained. However, the cellulose acetates with less than 54.1 or more than 56.0 combined acetic acid cannot be used alone, unblended that is, without "usable" cellulose esters for the purpose of this invention.

Of the four commercial types of cellulose acetate butyrate which are presently available on the American market each of them in several viscosity grades, I can use the following types (not viscosity grades) straight, unblended: cellulose acetate-butyrate EAM-381, having 37% combined butyryl, 13% combined acetyl, 50% combined cellulose residue, the latter having 2% free hydroxyl; cellulose acetate-butyrate EAB-500 with 48% combined butyryl, 6% combined acetyl, 46% combined cellulose residue, containing 0.7% free hydroxyl.

Two other types of cellulose acetate-butyrate types, EAB-171 and EAB-272, cannot be used straight but can be used blended especially with type EAB-381. Half Second butyrate (cellulose acetate-butyrate), most frequently used in the present examples, is a EAB-381 type (see Examples 7 and 8 below). The chemical composition of EAB-171 is 17% combined butyryl, 29.5% combined acetyl and 53.5% combined cellulose residue with 1.5% free hydroxyl. EAB-272 has 26% combined butyryl, 20.5% combined acetyl, 53.5% combined cellulose residue with 2.5% free hydroxyl.

In accordance with one aspect of this invention it is desirable to use a cellulose ester solution which contains at least a minimum concentration of about 20% by weight and preferably in the range of 20 to 35% by weight. As noted above, the total solids content of the icicle solution may vary from 30 to 50% by weight of the total composition. The non-ester solids dissolved in the icicle solution may vary from about 8% to about 15% by weight of the total solution. The non-ester solids are added to help avoid shrinkage and impart flame resistance and other desirable properties such as clarity, transparency, reduced brittleness, etc. Chlorinated biphenyls such as the "Arochlors" and chlorinated paraffin are the most useful. Other useful additives are certain aryl sulfonamide formaldehyde resins, Santolite MHP (see Example 2 below), organic bromine, boron or phosphorous compounds.

The viscosity of the "icicle solutions" of the present invention as distinguished from the viscosity of the various cellulose esters used herein and expressed as described above, are difficult to determine because of the fast jelling of the solution. However, it may be stated that the viscosity of the "icicle solutions" will vary within the limits of 85 to 170 seconds and preferably in the range of 85 to

130 seconds. The optimum range appears to be between 100 to 130 seconds. This viscosity is expressed as the falling time for a  $\frac{5}{16}$  in. steel ball through 10 in. of solution contained in a 1 in. wide tube at 25° C. and 760 mm. of Hg.

The following examples are further illustrative of the present invention and it will be understood that the invention is not limited thereto.

#### Example 1

36 p.p.w. (parts by weight) cellulose butyrate acetate ( $\frac{1}{2}$  sec.) and 11 p.p.w. chlorinated paraffin (40% chlorine) are dissolved in 53 p.p.w. methylenechloride. To 100% parts p.w. of this solution 18 parts p.w. of carbon-tetrachloride are gradually added under slow agitation.

*Remarks.*—This water clear, non-inflammable viscous liquid is free flowing; when a quantity of about  $\frac{1}{2}$  to  $\frac{3}{4}$  of one ounce of this liquid is squeezed at room temperature onto the end of a tree branch through the opening of a 20 collapsible metal tube, said opening having a diameter of  $\frac{1}{4}$  inch, this liquid will flow downwards in a cone-like shape until it has reached a length of about 3 to 4 inches. Sudden gelation and hardening of the surface at room temperature will stop any further movement or change of shape. The icicle-like product will become thoroughly rigid within a short time. It is odorless and will not burn if exposed to the open flame of a match.

#### Example 2

30 22 p.p.w. of cellulose acetate 8 sec., 8.8 p.p.w. Aroclor 1254 (chlorinated biphenyl), 4.2 p.p.w. Santolite MHP (arylsulfonamide formaldehyde resin) are dissolved in a blend of 58.5 p.p.w. methylenechloride and 6.5 p.p.w. methanol.

*Remarks.*—The properties of the resulting liquid are similar as described in Example 1.

#### Example 3

30 p.p.w. cellulose butyrate acetate 1 sec., 10 p.p.w. Aroclor 1254 (chlorinated biphenyl) are dissolved in a blend of 54 p.p.w. methylenechloride and 6 p.p.w. ethanol.

*Remarks.*—The resulting solution has similar properties as described in Example 1.

#### Example 4

45 7 p.p.w. cellulose butyrate acetate 3 sec., 28 p.p.w. cellulose butyrate acetate  $\frac{1}{2}$  sec., 9 p.p.w. Aroclor 1254 (chlorinated biphenyl) are dissolved in a blend of 46 p.p.w. methylenechloride, 4 p.p.w. ethylenedichloride, 5 p.p.w. methanol, 1 p.p.w. cyclohexane.

50 *Remarks.*—The resulting solution has similar properties as described in Example 1.

#### Example 5

55 5 p.p.w. cellulose acetate 20 sec., 20 p.p.w. cellulose butyrate acetate 1 sec., 8 p.p.w. Aroclor 1254 (chlorinated biphenyl) are dissolved in a blend of 60.3 p.p.w. methylenechloride and 6.7 p.p.w. methylalcohol methanol.

*Remarks.*—The resulting solution has similar properties as described in Example 1.

#### Example 6

60 35 p.p.w. cellulose butyrate acetate  $\frac{1}{2}$  sec., 11 p.p.w. Aroclor 1254 (chlorinated biphenyl), 4 p.p.w. Santolite MHP (arylsulfonamide formaldehyde resin) are dissolved in a blend of 45 p.p.w. methylenechloride and 5 p.p.w. methanol.

The cellulose acetate in Examples 2 and 5 has about 39% acetyl which is equal to a combined acetic acid of 54.2%. The cellulose butyrate acetate in Examples 1, 3, 5 and 6 has 37% combined butyryl, 13% combined acetyl, 50% combined cellulose residue, the latter having 2% free hydroxyl. The 3 second cellulose butyrate acetate in Example 4 is just inbetween a di- and tri-ester or, more precisely, contains 26% combined butyryl, 20.5% com-

53.5% combined cellulose residue with 2.5% free hydroxyl.

Examples 7 and 8

|                                                     | Percent by Wt. | Percent by Wt. |
|-----------------------------------------------------|----------------|----------------|
| Cellulose acetate butyrate 331-20                   | 6.5            | 7.5            |
| "Half second butyrate" (Cellulose acetate butyrate) | 25.5           | 26.5           |
| Aroclor 1254 (chlorinated biphenyl)                 | 10             | 10             |
| Solvent                                             | 58.0           | 56             |

The solvent in these examples consists of:

86% by wt. of methylene chloride  
4% by wt. of methanol  
5% by weight of ethanol  
3% by wt. of isopropanol  
2% by wt. of n-propanol

Both cellulose acetate butyrates in these examples have a combined butyryl content of 37%, a combined acetyl content of 13%, combined cellulose residue of 50% with a 2% free hydroxyl residue.

These formulas have a viscosity as measured above of 88 to 93 seconds. The solutions flow to an "icicle" that is of a length of from 3 to 7 inches before jelling and dry without even temporary blushing under dry or humid conditions and are easy to operate during the production.

Example 9

Percent by wt.

|                                                     |    |
|-----------------------------------------------------|----|
| Cellulose acetate PM-3 (Hercules)                   | 9  |
| "Half second butyrate" (cellulose acetate butyrate) | 21 |
| Aroclor 1254 (chlorinated biphenyl)                 | 10 |
| Methanol                                            | 6  |
| Methylene chloride                                  | 54 |

While the invention has been described with particular reference to specific embodiments, it is to be understood that it is not limited thereto, but is to be construed broadly and restricted solely by the scope of the appended claims.

I claim:

1. A viscous solution which is liquid and free flowing at normal room temperature in a closed container and which increases in viscosity rapidly and spontaneously to a point of gelation when released from said container and exposed to air at room temperature and normal atmospheric pressure consisting of a non-inflammable, high evaporation rate solvent system consisting of methylene chloride and a secondary solvent selected from the group consisting of methanol, ethanol, n-propanol, isopropanol, cyclohexane, carbontetrachloride, ethylene dichloride and

mixtures thereof, and a cellulose ester component dissolved therein, the ratio of methylene chloride to secondary solvent being in the range of from about 9.3:0.7 to 8:2, said methylene chloride and secondary solvent having a substantial difference in vapor pressure, said solvent system having a vapor pressure in the range of about 30 mm. to 360 mm. of Hg. at 20° C., said cellulose ester component containing as a principal and essential constituent a cellulose ester selected from the group consisting of cellulose acetate having an acetyl content of from 39 to 40.35% and a viscosity of from 1 to 8 seconds, cellulose acetate-butyrate having 6% combined acetyl and 48% combined butyryl content and cellulose acetate-butyrate having 13% combined acetyl and 37% combined butyryl content, said solution having a total solids content of from about 30% to 50%.

2. A viscous solution according to claim 1 wherein said solution has a viscosity of from 85 to 170 seconds.

3. A viscous solution according to claim 1 wherein the total cellulose ester component comprises at least 20% by weight of the solution.

4. A viscous solution according to claim 3 wherein the total cellulose ester component comprises from about 20% to 35% by weight of the total composition.

5. A viscous solution according to claim 1 wherein the ratio by weight of methylene chloride to secondary solvent is about 9:1.

6. A viscous solution according to claim 1 wherein cellulose esters enumerated constitute from 50% to 100% of said ester component.

7. A viscous solution according to claim 1 including a modifier selected from the class consisting of chlorinated biphenyl, chlorinated paraffins and arylsulfonamide formaldehyde resin.

8. A viscous solution according to claim 7 wherein said modifier is present in solution in the range of about 8% to 15% by weight of the total solution.

9. A process for making artificial icicles suspended directly from a support which comprises placing a small quantity of the composition of claim 1 on said support and allowing said composition to flow downwardly under the influence of gravity whereby an artificial icicle is formed.

References Cited in the file of this patent

UNITED STATES PATENTS

|           |                |               |
|-----------|----------------|---------------|
| 2,003,655 | Reid           | June 4, 1935  |
| 2,367,503 | Hunter et al.  | Jan. 16, 1945 |
| 2,492,978 | Fordyce et al. | Jan. 3, 1950  |
| 2,669,521 | Bierny         | Feb. 16, 1954 |
| 2,680,691 | Olson et al.   | June 8, 1954  |
| 2,739,070 | Fordyce et al. | Mar. 20, 1956 |